

1

3,395,052

## PRETREATING PROCESS FOR PHOSPHATE-TREATING STEEL SHEETS AND PLATED STEEL SHEETS

Shigeru Yonezaki, Minoru Kamada, Kazukiyo Terayama, and Katsunori Kanechika, Kitakyushu, Japan, assignors to Zawata Iron & Steel Co., Ltd., Tokyo, Japan, a corporation of Japan

No Drawing. Filed Sept. 9, 1964, Ser. No. 395,285

Claims priority, application Japan, Sept. 30, 1963,

38/52,940

14 Claims. (Cl. 148—6.15)

### ABSTRACT OF THE DISCLOSURE

The present invention provides for a method of phosphatizing the surface of steel sheets or plated steel sheets, wherein said method is preceded by a pretreating process, the improvement according to which the pretreating process comprises applying to the surface of said steel sheets, a liquid suspension of an insoluble phosphate selected from the group consisting of zinc phosphate, calcium phosphate, magnesium phosphate, ferrous phosphate, ferric phosphate, and aluminum phosphate.

This invention relates generally to pretreating processes for phosphate-treating the surface of ferrous metals and more particularly to economical pretreating processes for depositing phosphate films on steel sheets or plated steel sheets very quickly and compactly.

The present invention is a pretreating process to be carried out before phosphate films are applied to steel sheets or plated steel sheets such as galvanized steel sheets and comprises treating the surfaces of such steel sheets or plated steel sheets with a suspension of an insoluble phosphate of bivalent or trivalent metal. If such pretreatment is applied, in the subsequent phosphate treatment, a phosphate film will be produced within a very short time and will be very fine and compact.

Generally, in depositing a phosphate film on the surface of a steel sheet or plated steel sheet, the pretreatment of the surface is so important that, if no pretreatment is applied at all, no film will be produced at all or only a phosphate film of coarse crystals will be obtained in the subsequent phosphate treatment. It seems to be substantially ineffective to pretreatment to use a solution prepared by dissolving such soluble phosphate as, for example,  $Zn(H_2PO_4)_2$ .

Currently, the prior art has adopted a pretreating liquid comprising a solution of soluble sodium phosphate containing titanium. However, as a result of investigations we have made, it has been disclosed that the ingredient contributing to the formation of a phosphate film of fine crystals is the titanium in the solution. Further, with the decrease of titanium, we have found that the pretreating solution will be aged, that is, the coating weight of phosphate will increase and the crystal grains of the phosphate film will become coarse. As a result of the aging process the soluble phosphate in such pretreating liquid is not effective.

In order to obtain a suitable phosphate film by the above described prior art methods, the pretreating liquid must be frequently replaced so that a fixed amount of titanium may be always present. Thus this conventional pretreating liquid has decided disadvantages in that it is troublesome and costly.

Further, with such pretreating liquid, as described above, in order to form very fine phosphate film crystals on a steel sheet or a plated steel sheet, the concentration

2

of the liquid must be high and therefore the unit price of the product is much higher than that of the present invention. Even if the concentration of the liquid is kept high and the steel sheet is treated in said pretreating liquid and then further in a phosphate-treating liquid, the crystal size of the phosphate film will be almost invariably above  $3\mu$  and rarely below  $1\mu$ .

The prior art also utilizes a mechanical pretreating process wherein no pretreating liquid is used therein. According to this process, the surface of a steel sheet is rubbed with a proper rubbing tool before it is dipped in a phosphate-treating liquid. However, in such mechanical process, in order to carefully uniformly rub the surface of the steel sheet, a device of a considerably high precision is required. Therefore, it can not be recommended.

The present invention is designed to eliminate the defects of the prior art processes as described above. As a result of our research for a very economical and efficient pretreating process, we have now invented a new pretreating process for phosphate treatment.

According to the present invention, a suspension of an insoluble phosphate of a bivalent or trivalent metal is used so that the surface of a steel sheet may be mechanically rubbed and ground, and fine crystal nuclei of the phosphate may be then imparted to the surface thereof. Thus by the present invention, fine crystals of the phosphate may be produced uniformly on the surface of the steel sheet within a very short time.

An object of the present invention is to provide a pretreating process for the phosphate treatment of metal surfaces wherein a favorable fine compact phosphate film can be formed within a very short time on the surface of a steel sheet or a plated steel sheet such as a galvanized steel sheet.

Another object of the present invention is to provide a pretreating liquid which is economical and easy to apply by spraying or dipping in a pretreating process for phosphate-treating steel sheets or plated steel sheets.

Other objects and a fuller understanding of the invention may be had by referring to the following description and claims.

The present invention shall be described in detail in the following.

In the pretreating process according to the present invention, there is used an insoluble phosphate of a bivalent or trivalent metal suspended in water. For example, the insoluble phosphate of the bivalent metal is zinc phosphate, calcium phosphate, magnesium phosphate or ferrous phosphate and that of the trivalent metal is ferric phosphate or aluminum phosphate. In the case of a low concentration (up to about 3 g./liter), if the suspension is sprayed onto the surface of a steel sheet or a plated steel sheet under a high pressure, a favorable uniform pretreated surface will be obtained. In order to obtain a favorable result with a liquid of a high concentration, usually the steel sheet or plated steel sheet is dipped in the liquid or, after the dipping, the deposited liquid is pressed or rubbed onto the surface of the sheet with a roll or the like.

In the above mentioned spraying method under a high pressure, the favorable concentration of the suspension is more than 1 g./liter. However, if there is no restriction to the spraying manner, the higher the concentration, the better the result. Specifically a concentration of more than 5 g./liter is preferable. A proper concentration may be selected in response to the performances of the nozzle.

A spraying pressure of more than 0.5 kg./cm.<sup>2</sup> is preferable. The higher the spraying pressure, the better the result. Also, the longer the spraying time, the better the

result. But a spraying time of less than 1 minute is sufficient.

The spraying pressure, the spraying time and the concentration of the suspension are so closely correlated with one another that, when the spraying pressure is restricted, and the spraying time is made longer, a favorable result will be obtained and, when the spraying time is restricted, and the concentration of the suspension is elevated, a favorable result will also be obtained.

The above mentioned high pressure spraying method is effective to a suspension of a low concentration. But, when the concentration of the suspension is high, said method will be difficult to apply in view of the equipment. In the case of a suspension of such high concentration, only dipping the steel sheet in the suspension will be effective. Further repeating the dripping or squeezing with a roll after the dipping is effective.

The preferable pH of the suspension is slightly acid or alkaline at about 3 to 10. Outside this range, the steel sheet will corrode or will dissolve in the phosphate with an unfavorable result. It is proper to adjust the pH with phosphoric acid or sodium phosphate.

The bivalent or trivalent metal which is the principal agent in the present pretreating process may be used as crushed from crystals or as prepared from a soluble salt of the bivalent or trivalent metal or by adding a phosphate to the carbonate or oxide of such metal.

In the present invention, the higher the treating temperature, the better the result. But the effect of the temperature is rather small. Thus the treatment may be applied at 10 to 90° C.

When no pretreatment is applied at all, the crystal size of the obtained phosphate film will be so coarse as to be more than 100 $\mu$  but, when the present pretreatment is applied, the crystal size will be so fine as to be 2 $\mu$  or less. The time required to complete the phosphate treatment will be generally less than 2 minutes when the conventional pretreating process is carried out but will be so short as to be specifically less than 10 seconds when the present pretreating process is carried out.

Examples of the present invention are as follows:

#### Example 1

A fabricated steel sheet was dipped in an alkali solution so as to be degreased, was washed with water and was sprayed under the following conditions:

Ferric phosphate \_\_\_\_\_ g./liters\_ 30  
Liquid temperature \_\_\_\_\_ ° C.\_ 35  
pH \_\_\_\_\_ 9.8  
Spraying pressure \_\_\_\_\_ kg./cm.<sup>2</sup> 3.0  
Spraying time \_\_\_\_\_ minutes\_ 1

After the spraying treatment, the fabricated steel sheet was washed with running water and was then treated with phosphate-treating bath.

The time required to complete the phosphate treatment was only 10 seconds when the pretreatment of the present invention had been applied but was more than 5 minutes, sometimes no film being produced, when no pretreatment had been applied at all. The crystal size of the produced phosphate film was so fine as to be 2 $\mu$  when the present pretreatment had been applied.

#### Example 2

An electrogalvanized steel sheet was sprayed under the following conditions:

Zinc phosphate \_\_\_\_\_ g./liters\_ 25  
Liquid temperature \_\_\_\_\_ ° C.\_ 30  
pH \_\_\_\_\_ 7.8  
Spraying pressure \_\_\_\_\_ kg./cm.<sup>2</sup> 2.5  
Spraying time \_\_\_\_\_ seconds\_ 5

After the spraying treatment, the sheet was squeezed with a roll and was soon treated with phosphate-treating bath.

When the present pretreatment had been applied, the time required to complete the phosphate treatment was about 10 seconds and the crystal size of the produced phosphate film was so fine as to be 1 $\mu$ .

5

#### Example 3

A hot-dipped galvanized steel sheet was dipped under the following conditions:

Zinc phosphate \_\_\_\_\_ g./liters\_ 200  
10 Liquid temperature \_\_\_\_\_ ° C.\_ 70  
pH \_\_\_\_\_ 8.3  
Dipping time \_\_\_\_\_ seconds\_ 15

15

After the dipping treatment, the sheet was squeezed with a rubber roll, was washed with water and was treated with phosphate-treating bath.

20

When the present pretreatment had been applied, the time required to complete the phosphate treatment was about 15 seconds and the crystal size of the produced phosphate film was so fine as to be 2 $\mu$ .

25

While the present invention has been specifically described herein with reference to the preferred embodiments of the invention, it is to be understood that the present invention may be otherwise practiced than as specifically described within the scope and spirit of the appended claims.

What we claim is:

1. In a method of phosphatizing the surface of steel sheets or plated steel sheets, wherein said method is preceded by a pretreating process, the improvement according to which the pretreating process comprises applying to the surface of said steel sheets, a liquid aqueous suspension of an insoluble phosphate selected from the group consisting of zinc phosphate, calcium phosphate, magnesium phosphate, ferrous phosphate, ferric phosphate, and aluminum phosphate, in which said liquid suspension contains more than 1 g./l. of said phosphate and wherein the pH of the liquid is adjusted to from 3 to 10.
2. A process according to claim 1 wherein the suspension is sprayed onto the surface of the steel sheet under a spraying pressure of more than 0.5 kg./cm.<sup>2</sup>.
3. A process according to claim 2 wherein the temperature of the liquid suspension is 10 to 90° C.
4. A process according to claim 1 in which the steel sheet is dipped in the suspension of the insoluble phosphate during the pretreating process.
5. A process according to claim 4 in which the temperature of the liquid suspension is from 10 to 90° C.
6. A process according to claim 5 in which the steel sheets, after the pretreatment process are then squeezed with a roll.
7. A process according to claim 1 in which said insoluble phosphate is zinc phosphate.
8. A process according to claim 1 in which the insoluble phosphate is calcium phosphate.
9. A process according to claim 1 in which the insoluble phosphate is magnesium phosphate.
10. A process according to claim 1 in which the insoluble phosphate is ferrous phosphate.
11. A process according to claim 1 in which the insoluble phosphate is ferric phosphate.
12. A process according to claim 1 in which the insoluble phosphate is aluminum phosphate.
13. In a method of phosphatizing the surface of steel sheets or plated steel sheets, wherein said method is preceded by a pretreating process, the improvement according to which the pretreating process comprises dipping said steel sheets in a liquid aqueous suspension, containing at least 1 g./l. of zinc phosphate at a liquid temperature of 10 to 90° C. and at a pH of 3 to 10, then squeezing the sheets with a roll.
14. In a method of phosphatizing the surface of steel sheets or plated steel sheets, wherein said method is preceded by a pretreating process, the improvement according to which the pretreating process comprises spraying

75

a liquid aqueous suspension, containing at least 1 g./l. of zinc phosphate, at a liquid temperature of 10 to 90° C., onto the surface of said steel sheets, said spraying pressure being at least 0.5 kg./cm.<sup>2</sup> and the pH of said liquid being from 3 to 10.

|           |        |                |       |            |
|-----------|--------|----------------|-------|------------|
| 2,357,269 | 8/1944 | Russell et al. | ----- | 148—6.15 X |
| 2,479,423 | 8/1949 | Snyder         | ----- | 148—6.15   |
| 2,501,846 | 3/1950 | Gifford        | ----- | 148—6.15   |
| 2,514,149 | 7/1950 | Amundsen       | ----- | 148—6.15   |

## FOREIGN PATENTS

21,870 10/1963 Japan.

## References Cited

## UNITED STATES PATENTS

|           |        |            |       |          |
|-----------|--------|------------|-------|----------|
| 2,329,065 | 9/1943 | Lum et al. | ----- | 148—6.15 |
| 2,342,738 | 2/1944 | Jernstedt  | ----- | 148—6.16 |

ALFRED L. LEAVITT, *Primary Examiner.*  
R. L. BROWDY, *Assistant Examiner.*